

# UNITED STATES PATENT OFFICE.

ALFRED REGINALD McMULLEN, OF TORONTO, ONTARIO, CANADA.

## WOOD-POLISH.

1,067,359.

Specification of Letters Patent.

Patented July 15, 1913.

No Drawing.

Application filed November 21, 1912. Serial No. 732,683.

*To all whom it may concern:*

Be it known that I, ALFRED REGINALD McMULLEN, of the city of Toronto, in the county of York, in the Province of Ontario, Canada, have invented certain new and useful Improvements in Wood-Polishes, of which the following is the specification.

My invention relates to improvements in wood polishes, and the object of the invention is to devise a polish, which will be durable, comparatively cheap and most effectual in removing scratches or other blemishes on furniture and give the furniture a lasting and lustrous polish.

My invention consists of the following ingredients in the proportions set forth viz: One half gallon of raw linseed oil, one half gallon of turpentine, four ounces of sulfuric ether, eight drams by liquid measure of water ammonia, eight drams of dragons' blood. These proportions mixed together produce one imperial gallon. I merely state the proportions for a gallon, but it will be understood that in larger quantities the proportion will be the same.

In practice I beat the oil and turpentine

together and then add the sulfuric ether and then the ammonia and dragons' blood crushed to a fine powder, and thoroughly mix. In using my polish it should be thoroughly shaken.

A polish as above described produces a durable wearing surface that retains, and brings out the natural grain of the wood. It is essential in my polish that raw linseed oil be used and not boiled linseed oil as my polish would not be effectual with the boiled linseed oil.

What I claim as my invention is.

A wood polish comprising one-half gallon or thereabout of raw linseed oil, one-half gallon or thereabout of turpentine four ounces or thereabout of sulfuric ether, eight drams by liquid measure or thereabout of water ammonia, eight drams or thereabout of dragons' blood all mixed together as specified.

ALFRED REGINALD McMULLEN.

Witnesses:

B. BOYD,  
M. EGAN.

Copies of this patent may be obtained for five cents each, by addressing the "Commissioner of Patents, Washington, D. C."